

Patented May 5, 1925.

1,536,254

# UNITED STATES PATENT OFFICE.

CLARENCE B. WHITE, OF MONTCLAIR, NEW JERSEY, ASSIGNOR TO FRED S. BENNETT, INC., OF NEW YORK, N. Y., A CORPORATION OF NEW YORK.

WATER-REPELLENT TEXTILE MATERIAL AND METHOD OF PRODUCING THE SAME.

No Drawing.

Application filed December 9, 1922. Serial No. 605,984.

To all whom it may concern:

Be it known that I, CLARENCE B. WHITE, a citizen of the United States of America, residing at Montclair, in the county of Essex and State of New Jersey, have invented certain new and useful Improvements in Water-Repellent Textile Material and Methods of Producing the Same, of which the following is a full, clear, and exact description.

This invention relates to waterproofed and preserved textile materials and to methods of preparing the same, more particularly materials in which the fibres thereof are impregnated, coated, or otherwise treated with compounds of rare earth metals such as thorium, cerium, lanthanum, didymium (neodymium and praseodymium), zirconium and uranium. The chief object of the invention is to provide textile materials which are not only highly repellent to water but which are not materially impaired in that quality by treatment with gasoline, benzene, naphtha, and other hydrocarbons such, for example, as are employed in so-called "dry-cleaning". In carrying out the invention in the preferred manner the substances used for giving the fabric or other fibrous material the desirable properties of water-repellency, resistance to injurious influences of atmospheric gases, etc., are what may for convenience be termed metallic soaps of the rare earths, that is, fatty-acid salts of such elements; and especially salts of the higher organic acids and their derivatives, for example acids of the general type  $C_nH_{2n}O_2$ ; the oleic series, type  $C_nH_{2n}2O_2$ ; the linoleic series, type  $C_nH_{2n}4O_2$ ; the linolenic series, type  $C_nH_{2n}6O_2$ ; the chaulmoogric cyclic series, type  $C_nH_{2n}8O_2$ . Of the compounds of rare earth elements and acids of the kind indicated, such metallic soaps as oleates, linoleates, alpha-elæostearates, and abietates are in general, when freshly precipitated, fairly soluble in heated ether, turpentine, gasoline, etc., while metallic soaps of the higher acids, for example stearates, elaidates, beta-elæostearates, and palmitates are only very sparingly soluble in ether, hot or cold, and still less so in turpentine, gasoline, benzene, and other liquid hydrocarbons. Such salts are also highly resistant to alkali, whether caustic or carbonate, and when decomposed thereby, if at all, they are converted into insol-

uble hydroxides or carbonates. For example, the fatty acid soap cerium palmitate is almost completely insoluble in turpentine and benzol, and in hot ether is soluble only to the extent of about 0.8 per cent. 60

Heretofore, aluminum hydroxid or aluminum soap has been used to give water-repellency to textile materials, but each of these compounds is readily converted, on coming into contact with free alkali, into soluble sodium or potassium aluminate, which is removed by the action of water, thus destroying or seriously impairing the water-proof property of the fabric. This is not the case, however, with the metallic soaps of the rare earth elements, inasmuch as these are not removed by free caustic alkalis. In the case of carbonate alkalis, double carbonates of the rare earths are sometimes formed to a limited extent, but these carbonates, with the possible exception of the thorium and zirconium salts, are not soluble in the re-agent and hence remain in the fabric, which therefore retains its water-repellent quality. 70 75 80

This characteristic of the salts of rare earth elements, namely, their relative inertness to alkalis, renders them especially advantageous for the treatment of textile materials to make the same water-repellent, or to serve as mordants for dyes or form insoluble lakes on the fibre. Moreover, they are antiseptic in character, and hence resist mildew and spore growth, which further distinguishes them from aluminum salts in 85 general use for treating fabrics. 90

As explained in my copending application Serial No. 639,219, when a fabric has been treated with a soluble metallic salt which is absorbed by the fibres thereof, and the salt has been converted by chemical or electrolytic action into an insoluble compound, as for example into a hydroxid, phosphate, fluorid, chromate, tungstate, stannate, etc., the fabric becomes repellent 95 to water. This repellency appears to be "internal", that is, due to an actual absorption by the fibres, rather than "surface repellency" produced by coating the fibres. I have discovered that if a fabric so treated be again treated with a metallic salt, preferably a rare earth salt, and this salt be converted into an insoluble compound, the fabric has imparted to it a high degree 100 of surface repellency and also has its in- 105 110

ternal repellency increased. Moreover, the capillarity of the fabric is almost if not wholly destroyed. In one of these treatments an aluminum salt may be used, with or without a rare earth salt in the same treatment, for the reason that the presence of the rare earth in one or both coatings or impregnations renders the aluminum salt much more stable and difficult of removal from the fibre by caustic alkali.

In carrying out my invention, advantage may be taken of the fact, stated above, that freshly precipitated oleate, linoleate, abietate, etc., are soluble in hydrocarbon solvents, especially when the solvent is hot. Hence the desired treatment can be affected by passing the fabric or fibres (or, in general, the textile material) through a warm or hot solution of the selected metallic soap or soaps in gasoline, benzene, carbon tetrachlorid, tetrachlorethane, or the like, and then drying the material. With the rare earth metallic soaps of higher fatty acids, however, the procedure is, in general, less simple. In such cases the double treatment may be employed,—first with a soluble metallic soap of these acids, as for example the stearate, palmitate, elaidate, etc., of sodium, potassium or ammonium, and then with a solution (or an emulsion) of an inorganic salt or other compound of a rare earth metal or metals, as for example chlorid of cerium, thorium, or lanthanum, etc., or acetate, formate, sulfate, sub-nitrate, or chlorid of one or more of such metals. As a result, an insoluble fatty acid compound of the metal or metals is formed or precipitated in the textile material, rendering the latter highly repellent to water, non-capillary, and capable of being washed with soap and of being cleaned with gasoline and other hydrocarbon agents without loss of its water-repellency. Of course, in this double treatment, fatty acid soaps of the rare earth metals which are soluble in hydrocarbon solvents, as for example oleates, linoleates, etc., may be used if desired.

In some cases the soluble metallic soap or soaps used may be replaced by an emulsion of a fatty acid compound, as for example an emulsion of Japan wax. To such emulsions rubber, paraffin, ceresin, or other wax capable of being emulsified, can be added, which will be deposited on the fibres or within the pores thereof without thereby interfering with the reaction between the metallic soap and the solution with which the fabric is afterwards treated.

It is not essential, in all cases, that the textile material be treated first with the soap compound, inasmuch as excellent results can be obtained by reversing the order; impregnating in the first instance with the soluble salt and then passing the material

through the soap solution. In this order of treatment, however, the acid salts employed (say the chlorid, acetate, sulfate, etc.) have a tendency to precipitate the soap or break the emulsion and as a result the fabric or fibres are apt to be marred by deposition of flakes of soap or by solid particles of the emulsion, especially where waxes or rubber compounds are used in the emulsion.

An alternative mode of depositing a metallic soap upon or within the fibres is to first deposit the metallic element in the form of an insoluble compound which is decomposable by a fatty acid, as for example a carbonate or hydroxid of the selected metal or metals, and then treat the material with a fatty acid, or acids, such as oleic, stearic, palmitic, etc., with resulting conversion of the carbonate or hydroxid into the corresponding fatty acid salt or metallic soap. In this procedure the deposition of the insoluble compound can be effected by the method described in my copending application above mentioned.

In general, metallic soaps can be deposited: (1) By direct deposition from a solution; (2) By the action of a fatty acid, such as stearic, oleic, palmitic, etc., upon rare earth carbonate or hydroxid freshly precipitated on or in the fibres; and (3) By the interaction of soluble rare earth salt (say a chlorid, acetate, sulfate, etc.) and an alkali salt of the desired fatty acid, as for example sodium, potassium or ammonium stearate, palmitate, oleate, elaidate, etc. In the second of these methods the resulting salts are almost invariably of an acid type; while in the second, which depends upon double decomposition, normal neutral salts are produced if precautions are taken to avoid excess of the rare earth salt or of the fatty acid salt.

For some purposes it is advantageous to first deposit on the fibres an insoluble rare earth compound, such as a carbonate, hydroxid, phosphate (or tho-, meta-), hypophosphate, etc., preferably carbonate, hydroxid or phosphate. This gives the subsequently deposited metallic soap an underlying basis which is itself repellent and capable of neutralizing or resisting to a considerable extent at least, the action of atmospheric gases, such as carbon dioxide and traces of sulfuric and nitric acids. The fabric is thus able to resist the destructive influences of such atmospheric agencies to a much greater degree than is an untreated fabric. When fabric is painted and thereby impregnated with drying oils, slow hydrolysis takes place, especially when exposed to light, and the drying oils set free organic acids which attack the fibre. If there is an underlying metallic hydroxid or carbonate (for example) the fatty acid combines therewith to form a metallic soap.

and hence does not attack the fibre. For certain purposes, as for example roofing material, the presence of this underlying metallic compound is especially important, 5 as it has a marked protective effect against the destructive action of air, light and moisture. The desired insoluble rare earth compound can be deposited on the fibres by first treating with a soluble rare earth salt, 10 say a chlorid, acetate, or nitrate, drying the material; and then treating with an alkaline carbonate, hydrate, sulfid, or the like. After this treatment (in which double decomposition takes place) the material can be 15 freed from alkalin salts by washing with water. In some cases a rare earth phosphate is advantageous as the underlying coating; such phosphates being in general very insoluble and tending to make dyes 20 faster, especially direct dyes.

Various ways of carrying out my invention in practice will now be given; it being understood, however, that the invention is not limited to the specific details or materials set forth. In general the fabrics (or fibres, as the case may be) need not be subjected to treatment longer than is necessary for thorough wetting, after which they are dried, being first squeezed to eliminate as 25 much as possible of the treating liquid or emulsion, in order to avoid loss, as by evaporation.

(A) For direct deposition of metallic soap: A ten per cent solution of cerium, 30 thorium, lanthanum or didymium oleate or linoleate, in varnoline or gasoline. Use warm.

(B) For impregnation and proofing by double decomposition: (1) Stearate of sodium, five per cent aqueous solution. Use hot. Impregnate the textile material, dry the same, and pass through five per cent aqueous solution of cerium or thorium acetate. (2) Five per cent aqueous solution 40 of a mixture composed of cerium acetate two parts (by weight), lanthanum acetate one part, didymium acetate one part. Dry, and pass through five per cent solution of sodium, potassium or ammonium stearate 45 or palmitate.

(C) With an emulsion of Japan wax (largely stearic and palmitic acids): Ten per cent emulsion in water at about 140° F. Impregnate, squeeze, and pass through 50 five per cent aqueous cold solution of thorium acetate-nitrate; or through hot or cold five per cent solution of acetate (or chlorid, sulfate, etc.) of cerium two parts, of lanthanum one part, and of didymium one part.

(D) Stearic acid twenty-six parts, oleic acid 12 parts, paraffin thirty-six parts, saponified with caustic soda twenty-six 55 parts; in eight hundred parts water. Impregnate, and pass through either of the

solutions mentioned above for the second treatment in Example (C).

(E) Proofing upon a prepared base of rare earth hydroxid, carbonate or phosphate; pass the material through a five to 70 ten per cent solution of a soluble salt of thorium (or cerium, lanthanum, or didymium, etc.), squeeze and dry; pass through a solution of alkalin hydrate (sodium, potassium or ammonium hydrate), rinse and 75 dry; pass through five per cent solution of sodium stearate, then through five per cent solution of cerium (or lanthanum or didymium) acetate, wash, and dry. Or: Pass the material through a five to ten per cent 80 solution of a soluble thorium salt or its equivalent in cerium, lanthanum and (or) didymium. Dry, and pass through alkalin hydrate or sulfid solution, wash and dry. Impregnate with emulsion of Japan wax 85 (say ten per cent) at 140° F., and then pass through a five per cent solution of a rare earth salt. Or: Pass through a five to ten per cent solution of a rare earth salt, dry and pass through a hot ten to fifteen per 90 cent solution of ammonium, sodium or potassium phosphate, squeeze, wash in water, and dry. Pass the dried material through a Japan wax emulsion (saponified) of a strength indicated by five to ten parts 95 in ninety-five to ninety parts water, at 140° to 150° F. Then pass through a five per cent rare earth salt in water.

The invention is applicable to a large 100 variety of textile materials (using the latter to include woven, felted, knit, netted, and other fabrics, threads, yarns, warps, fibres, etc.) of vegetable or animal origin, as for example cotton, silk and wool.

It is to be understood that the invention 105 is not limited to the details herein described but can be carried out in other ways without departure from its spirit as defined by the appended claims.

I claim—

1. Water-repellent textile material impregnated with a fatty acid compound of a rare earth metal.

2. Water-repellent textile material impregnated with a metallic soap which is, 115 at most, sparingly soluble in hydrocarbons.

3. Water-repellent textile material impregnated with a rare earth compound of a fatty acid of the type  $C_nH_{2n}O_2$ .

4. Water-repellent textile material impregnated with an insoluble inorganic rare earth metal compound and with an insoluble organic rare earth metal compound.

5. A process of rendering textile material water-repellent, comprising impregnating 125 the material with a fatty acid compound of a rare earth metal.

6. A process of treating textile material to render the same water-repellent, comprising treating the material with a solution 130

of a fatty acid compound of an alkali metal, and with a solution of a salt of a rare earth metal.

7. A process of treating textile material to render the same water-repellent, comprising depositing on the fibres of the material an insoluble inorganic compound of a rare earth metal, and treating the material with a solution of a fatty acid compound of an alkali metal, and with a solution of an inorganic salt of a rare earth metal. <sup>15</sup>  
In testimony whereof I hereto affix my  
10 metal.

8. A process of treating textile material to

CLARENCE B. WHITE.